



US005658846A

**United States Patent** [19]

Slark

[11] **Patent Number:** **5,658,846**[45] **Date of Patent:** **\*Aug. 19, 1997****[54] THERMAL TRANSFER PRINTING DYE-SHEET****[75] Inventor:** **Andrew Trevithick Slark, Suffolk, England****[73] Assignee:** **Imperial Chemical Industries PLC, Great Britain****[\*] Notice:** The term of this patent shall not extend beyond the expiration date of Pat. No. 5,595,956.**[21] Appl. No.:** **387,883****[22] PCT Filed:** **Aug. 26, 1993****[86] PCT No.:** **PCT/GB93/01818**§ 371 Date: **Mar. 22, 1995**§ 102(e) Date: **Mar. 22, 1995****[87] PCT Pub. No.:** **WO94/04371**PCT Pub. Date: **Mar. 3, 1994****[30] Foreign Application Priority Data**

Aug. 26, 1992 [GB] United Kingdom ..... 9218126

**[51] Int. Cl.<sup>6</sup>** ..... **B41M 5/035; B41M 5/38****[52] U.S. Cl.** ..... **503/227; 428/195; 428/500; 428/913; 428/914****[58] Field of Search** ..... **8/471; 428/195, 428/500, 913, 914; 503/227****[56] References Cited****FOREIGN PATENT DOCUMENTS**A 0 179 737 4/1986 European Pat. Off. ..... 503/227  
A 0 453 020 10/1991 European Pat. Off. ..... 503/227  
0469723 2/1992 European Pat. Off. ..... 503/227  
A 0 474 197 3/1992 European Pat. Off. ..... 503/227**OTHER PUBLICATIONS**

Database WPI Week Week 8607, Derwent Publications Ltd., London, GB; AN 86-046114 &amp; JP A 61 000 692 (Oike Kogyo KK) 6 Jan. 1986.

*Primary Examiner*—Bruce H. Hess**[57] ABSTRACT**

A thermal transfer printing dye-sheet which comprises a substrate having on one side, a dye coat comprising a binder and a thermally transferable dye wherein the binder comprises a polymer, at least 10% of the monomeric units of the polymer being derived from parahydroxystyrene, the phenyl group of which may or may not be further substituted.

**17 Claims, No Drawings**

## THERMAL TRANSFER PRINTING DYE-SHEET

This invention relates to a thermal transfer printing (TTP) dye sheet, in particular to a dye sheet having an improved dye binder.

Thermal transfer printing is a printing process in which a dye is caused, by thermal stimuli, to transfer from a dye sheet to a receiver sheet thereby to form an image on the receiver sheet. In such a process, the dye sheet and receiver sheet are placed in intimate contact, the thermal stimuli are applied to the dye sheet to cause dye transfer and the dye sheet and receiver sheet are then separated. By applying the thermal stimuli to pre-determined areas in the dye sheet, the dye is selectively transferred to the receiver to form the desired image. The thermal stimuli may be provided by a programmable print head which is in contact with the dye sheet or by for example, a laser in a light-induced thermal transfer process (LITP).

Dye-sheets conventionally comprise a substrate having on one surface thereof a dye coat which typically comprises a thermally transferable dye dispersed or dissolved in a binder. Dye-sheets may also comprise a back coat to impart desirable properties for example, good handling and thermal characteristics to the dye sheet. Further, a primer or subbing layer may be employed between the substrate and the dye coat and/or the substrate and the back coat for example to improve the adhesion of the coat to the substrate.

Many materials have been suggested for use as the binder including, cellulosic polymers as disclosed in J03264393, polyvinylbutyral as disclosed in EP-A-141678, epoxy resins and phenolic resins. J59199295 discloses an ink composition for sublimation dye transfer consisting of cellulose acetate, polystyrene, a disperse dye, silica and methylethyl ketone.

During the TTP process, application of a thermal stimulus to an area of the dye coat of the dye sheet heats that area of the sheet to a temperature typically in excess of 100° C. as a result of which the dye in that area of the dye sheet is transferred to the receiver sheet. On removal of the thermal stimulus the temperature of the heated area then decreases to the ambient operating temperature in the process.

However, once the thermal stimulus is removed and the temperature of the heated area of the dye sheet is decreasing, there may be still be sufficient heat to cause unwanted, uncontrolled residual transfer of dye to the receiver sheet which may cause a reduction in image quality. This effect is known as low temperature thermal transfer.

We have now found that by employing a dye sheet binder comprising a polymer having a monomeric unit of an optionally substituted styrene provided that where unsubstituted styrene is present in the polymer then the polymer is a copolymer problems due to low temperature thermal transfer may be reduced or avoided and other significant advantages may also be secured.

Accordingly, a first aspect of the invention provides a thermal transfer printing dye sheet which comprises a substrate having on one side, a dye coat comprising a binder and a thermally transferable dye wherein the binder comprises a mixture of a polymer having, as at least 10% of the monomeric units of the polymer, a monomeric unit of formula (I);



(I)

wherein X is H or methyl and Y is an optionally substituted phenyl group, a cyano group or an ester group of formula  $-CO_2Z$  wherein Z is an optionally substituted  $C_1$  to  $C_6$

hydrocarbyl group with the proviso that where Y is an unsubstituted phenyl group the second polymer also has a substituted styrene and/or a non-styrene monomeric unit.

Dye-sheets according to the present invention have been found to exhibit a particularly advantageous combination of characteristics. In particular, good resistance to low temperature thermal transfer may be achieved which provides for improved image quality and images may be produced which have excellent optical density.

Also, we have found that when the dye sheet is to be used to produce multi-colour images by using a dye sheet comprising a plurality of panels of different uniform colours, usually magenta, yellow and cyan, improved colour balance between the dyes by matching the three colours may be achieved. A practical benefit of this is that an excess of one or more of the colours leading to a colour imbalance and hence a tinge of the image may be reduced or avoided, such imbalance being particularly undesirable and visually prominent in neutral colours for example grey.

The polymer may be a homopolymer, the monomeric unit of which is derived from parahydroxystyrene, the phenyl group of which may or may not be further substituted.

Alternatively, the polymer may be a copolymer (block, random, alternating or graft) and formed of monomeric units according to formula 1 where Y is substituted phenyl and monomeric units according to formula 1 where Y is unsubstituted phenyl or an ester group of formula  $-CO_2Z$  where Z is an optionally substituted  $C_1$  to  $C_6$  hydrocarbyl group, and/or monomeric units derived from maleic anhydride.

According to a further alternative, the polymer may be a copolymer formed of monomeric units according to formula 1 where Y is unsubstituted phenyl and monomeric units derived from maleic anhydride.

In another alternative, the polymer may be a copolymer formed of monomeric units according to formula 1 where Y is unsubstituted phenyl and monomeric units according to formula 1 where Y is an ester group of formula  $-CO_2Z$  where Z is an optionally substituted  $C_1$  to  $C_6$  hydrocarbyl group.

Preferably, the further substituent on the phenyl group is halogen (most preferably bromine), glycidyl neodecanoate, hydroxymethyl, dimethylaminomethyl, 2-hydroxyethylmethylaminomethyl, t-butyl, sulphonate, styrene or benzoate.

According to a further preferred feature, the hydrocarbyl group is hydroxyethyl, hydroxypropyl or hydroxybutyl.

A most preferred thermal transfer printing dye sheet comprises a substrate having on one side, a dye coat comprising a binder and a thermally transferable dye wherein the binder comprises a polymer selected from the group consisting of:

a parahydroxystyrene homopolymer,  
a bromo-parahydroxystyrene homopolymer,  
a copolymer of parahydroxystyrene and parahydroxystyrene further substituted with halogen (eg bromine), glycidyl neodecanoate, hydroxymethyl, dimethylaminomethyl, 2-hydroxyethylmethylaminomethyl, t-butyl, sulphonate, styrene or benzoate,

a copolymer of parahydroxystyrene with or without a further substituent on the phenyl group and any one or a mixture of methyl(meth)acrylate, 2-hydroxy(meth)acrylate, butyl (meth)acrylate, fluoro(meth)acrylate and acrylic acid

Where the polymer is a copolymer, suitably at least 10% and preferably at least 25% of the monomeric units of the polymer, based on the total number of monomeric units in

the polymer, are of formula (I). The two monomeric units are suitably present in a ratio in the range 15:85 to 85:15 and preferably 25:75 to 75:25.

The glass transition temperature (Tg) of the polymer is suitably in the range 50° C. to 200° C. and preferably 60° to 185° C.

The optionally substituted styrene polymer is suitably present in the dye-coat in an amount of at least 5% by weight of the total dye coat weight.

A further aspect of the invention provides a thermal transfer printing method which comprises placing a dye-sheet according to any aspect of the present invention in contact with a receiver sheet which comprises a substrate having on one side a dye-receptive surface, applying thermal stimuli to the dye-sheet at pre-determined locations to effect thermal transfer of the dye from the said locations to the dye-receptive surface thereby to form a pre-determined dye image and separating the dye-sheet and receiver sheet.

The dyecoat is formed by coating the substrate, or a layer on the substrate, with an ink prepared by dissolving or dispersing one or more thermal transfer dyes and the binder in a liquid vehicle to form a coating composition; then removing any volatile liquids. Any dye capable of being thermally transferred in the manner described above, may be selected as required. Dyes known to thermally transfer, come from a variety of dye classes, e.g. from such nonionic dyes as azo dyes, anthraquinone dyes, azomethine dyes, methine dyes, indoaniline dyes, naphthoquinone dyes, quinophthalone dyes and nitro dyes.

The ink may also include dispersing agents, antistatic agents, antifoaming agents, and oxidation inhibitors, and can be coated onto the substrate as described for the formation of the latter. The thickness of the dyecoat is suitably 0.1-5 µm, preferably 0.5-3 µm.

The dye and binder are suitably present in a weight ratio of 0.1 to 3:1 of dye:binder. The precise ratio of dye to binder will be determined by a consideration of the particular dye and binder to be employed and the application for which the dye sheet is intended to be used.

Preferably, the dye sheet comprises a backcoat disposed on the opposite side of the substrate to the dye-coat to provide suitable heat resistance and slip and handling properties. Suitable backcoats having a desirable balance of properties include those described in EP-A-314348 and especially those described in EP-A-458522. Particularly preferred backcoats include those in which the backcoat comprises the reaction product of radically co-polymerising in a layer of coating composition, the following constituents:

- a) at least one organic compound having a plurality of radically polymerisable saturated groups per molecule and
- b) at least one organic compound having a single radically polymerisable unsaturated group

the backcoat also containing an effective amount, as slip agent, of

- c) a metallic salt of a phosphate ester.

In cases, where the dye sheet is to be used in a LITT process, a light absorbing material may be included in the dye-coat or, if desired, a separate absorber layer comprising a light absorbing material disposed between the dye-coat and the substrate may be employed. The light-absorbing material suitably comprises a material which is an absorber for the inducing light to convert it into the required thermal energy to effect thermal transfer of the dye.

If present, the absorber is preferably carbon black, as this provides good absorption and conversion to heat, of a broad spectrum of wavelengths, and hence is not critical to the inducing light source employed for the printing, further, it is also relatively cheap.

However, any suitable absorber materials known in the art may be employed as desired. For lasers operating in the near infrared, there are also a number of organic materials known to absorb at the laser wavelengths. Examples of such materials include the substituted phthalocyanines described in EP-B-157,568, which can readily be selected to match laser diode radiation at 750-900 nm, for example.

A variety of materials can be used for the substrate, including transparent polymer films of polyesters, polyamides, polyimides, polycarbonates, polysulphones, polypropylene and cellophane, for example. Biaxially orientated polyester film is the most preferred, in view of its mechanical strength, dimensional stability and heat resistance. The thickness of the substrate is suitably 1-50 µm, and preferably 2-30 µm.

Various coating methods may be employed to coat the dye-coat and if present, other coats for example a backcoat, onto the substrate, including, for example, roll coating, gravure coating, screen coating and fountain coating. After removal of any solvent, the coating can be cured by heating or by irradiating with electromagnetic radiation, such as ultraviolet light, electron beams and gamma rays, as appropriate. Typical curing conditions are heating at 50°-150° C. for 0.5-10 minutes (in the case of thermal curing), or exposure to radiation for 1-60 s from an ultraviolet lamp of 80 W/cm power output, positioned about 15 cm from the coating surface (in case of ultraviolet light curing). In-line UV curing may utilise a higher powered lamp, eg up to 120 W/cm power output, focused on the coating as it passes the lamp in about 0.1-10 ms. The coating is preferably applied with a thickness such that after drying and curing the thickness is 0.1-5 µm, preferably 0.2-3 µm, and will depend on the concentration of the coating composition.

The dye sheet may be elongated in the form of a ribbon and housed in a cassette for convenience, enabling it to be wound on to expose fresh areas of the dyecoat after each print has been made.

Dyesheets designed for producing multicolour prints have a plurality of panels of different uniform colours, usually three: yellow, magenta and cyan, although the provision of a fourth panel containing a black dye, has also previously been suggested. When supported on a substrate elongated in the form of a ribbon, these different panels are suitably in the form of transverse panels, each the size of the desired print, and arranged in a repeated sequence of the colours employed. During printing, panels of each colour in turn are held against a dye-receptive surface of the receiver sheet, as the two sheets are imagewise selectively irradiated to transfer the dye selectively where required, the first colour being overprinted by each subsequent colour in turn to make up the full colour image.

The invention is illustrated by the following non-limiting examples.

#### EXAMPLE 1

A selection of dye sheets were produced by coating a dye coat of composition listed in Table 1 onto a 6 µm thick polyethylene terephthalate substrate having a subcoat (onto which the dye coat was coated) on one side and a back coat on the opposite side using a wire bar. For all the dye sheets the substrate, sub coat and back coat were the same. Once coated, the dye coat was dried in an oven for 20 seconds at 110° C. to produce a dye sheet having a dry dye coat thickness of 1 µm. Examples 1B, 1D and 1F illustrate the present invention and Examples 1A, 1C and 1E are comparative Examples according to the prior art.

TABLE 1

| Components        | *1A   | 1B    | *C   | 1D   | *1E   | 1F   |
|-------------------|-------|-------|------|------|-------|------|
| Dye C1            | —     | —     | 1.60 | 1.60 | —     | —    |
| Dye C2            | —     | —     | 1.60 | 1.60 | —     | —    |
| Dye M0            | 4.30  | 4.31  | —    | —    | 4.30  | 6.45 |
| Dye M3            | 1.07  | 1.08  | —    | —    | 1.07  | 1.62 |
| Ethyl cellulose   | 1.18  | —     | 4.50 | —    | 1.18  | —    |
| Polyvinyl butyral | 4.73  | —     | —    | —    | 4.73  | —    |
| S/PHS copolymer   | —     | 5.92  | —    | 4.50 | —     | —    |
| PPHS              | —     | —     | —    | —    | —     | 3.23 |
| Tetrahydro-furan  | 88.72 | 88.69 | 92.3 | 92.3 | 88.72 | 88.7 |

\*comparative Example

C<sub>1</sub> was 3-acetyl amino-4-(3-cyano-5-phenylazothiophenyl-2-ylazo)-N,N-diethyl aniline; C<sub>2</sub> was CI solvent blue 63; M0 was CI disperse red 60; M3 was 3-methyl-4(3-methyl-4-cyanoisothiazol-5-ylazo)-N-ethyl-N-acetoxyethyl aniline;

Ethyl cellulose was grade ECT-10 available from Hercules;

Polyvinyl butyral had a molecular weight of 100000, a Tg of 85° C. and was grade SLEC BX1 available from Sekisui;

S/PHS copolymer was a styrene/parahydroxystyrene copolymer and PPHS was polyparahydroxystyrene, both available from Hoechst Celanese.

## EXAMPLE 2

A receiver sheet was produced by coating onto a polyethylene terephthalate substrate having a backcoat and a subcoat, a dye-receptive layer of the following composition:

|                                                            |         |
|------------------------------------------------------------|---------|
| Vylon 200                                                  | 11.60%  |
| Tegomer HSi 2210                                           | 0.08%   |
| ((bis-hydroxyalkyl polydimethyl-siloxane from Goldschmidt) |         |
| Cymel 303                                                  | 0.16%   |
| Di-n-butyl amine blocked toluene 0.05%                     |         |
| sulphonic acid catalyst                                    |         |
| Tinuvin 234                                                | 0.12%   |
| (UV stabiliser)                                            |         |
| Toluene/Methyl ethyl ketone                                | to 100% |
| 47.5/52.5 solvent mixture                                  |         |

The dye-receptive coat was dried for 3 minutes at 140° C. to provide a dry coat thickness of 4 μm.

The dye sheets produced in Example 1 were each brought into contact with a sample of the receiver sheet and thermal transfer printing was effected by means of a programmable print head supplying heat pulses of 2 to 14 millisecond duration to the backcoat of the dye sheet to provide a gradation in the optical density of the print image. Printing in the case of Examples 1E and 1F was effected using a different printer. The dye sheet and receiver sheet were separated following printing and the reflection optical densities on the receiver sheet were measured using a Sakura densitometer and are shown in Table 2.

## EXAMPLE 3

In order to simulate the conditions under which unwanted low temperature thermal transfer under normal print conditions may occur, samples of the dye sheets produced in Example 1 and the receiver sheet produced in Example 2 were fed, in register, through a 2-roll laminator (OZATEC

HRL350 hot roll laminator available from Hoechst) at 0.2 ms<sup>-1</sup>. The rolls of the laminator were maintained at a temperature of 60° C. and the pressure between them was 5 bar. The reflection optical densities on the receiver sheet were measured using a Sakura densitometer and are shown in Table 2, the column headings denoting which dye sheet was used in the test.

TABLE 2

| Print Time (ms)                              | Optical Density |      |      |      |      |      |
|----------------------------------------------|-----------------|------|------|------|------|------|
|                                              | *1A             | 1B   | *C   | 1D   | *1E  | 1F   |
| 2                                            | 0.086           | 0.09 | 0.06 | 0.06 | —    | —    |
| 3                                            | 0.12            | 0.12 | 0.07 | 0.09 | 0.09 | 0.10 |
| 4                                            | 0.28            | 0.19 | 0.14 | 0.16 | 0.19 | 0.22 |
| 5                                            | 0.55            | 0.37 | 0.35 | 0.32 | 0.38 | 0.35 |
| 6                                            | 0.82            | 0.62 | 0.69 | 0.53 | 0.68 | 0.52 |
| 7                                            | 1.22            | 0.92 | 1.11 | 0.79 | 0.85 | 0.74 |
| 8                                            | 1.72            | 0.35 | 1.66 | 1.18 | 1.17 | 1.06 |
| 9                                            | 2.12            | 1.74 | 2.09 | 1.67 | 1.59 | 1.56 |
| 10                                           | 2.27            | 1.98 | 2.37 | 2.05 | 1.94 | 2.07 |
| Low Temperature Thermal Transfer (at 60° C.) | 0.36            | 0.18 | 0.24 | 0.14 | 0.28 | 0.14 |

\*comparative Example

The above results illustrate that significant reductions in dye transferred as a result of low temperature thermal transfer may be secured, by using dye sheets according to the present invention whilst maintaining acceptable optical densities in normal printing as compared with dye sheets of the prior art.

I claim:

1. A thermal transfer printing dye-sheet which comprises a substrate having on one side, a dye coat comprising a binder and a thermally transferable dye wherein the binder comprises a polymer, at least 10% of the monomeric units of the polymer being derived from parahydroxystyrene, the phenyl group of which may or may not be further substituted.

2. A dye-sheet according to claim 1, wherein the polymer is a homopolymer.

3. A dye-sheet according to claim 1, wherein the further substituent is a halogen, hydroxymethyl, dimethylaminomethyl, 2-hydroxyethylmethylaminomethyl or t-butyl.

4. A dye-sheet according to claim 3, wherein the halogen is bromine.

5. A dye-sheet according to claim 1 wherein the polymer comprises a copolymer formed of monomeric units according to formula 1 where Y is substituted phenyl and monomeric units according to formula 1 where Y is unsubstituted phenyl or an ester group of formula —CO<sub>2</sub>Z where Z is an optionally substituted C<sub>1</sub> to C<sub>6</sub> hydrocarbyl group, and/or monomeric units derived from maleic anhydride.

6. A dye-sheet according to claim 5, wherein the substituent on the phenyl group is hydroxy.

7. A dye-sheet according to claim 6, wherein the substituted phenyl group is further substituted.

8. A dye-sheet according to claim 7, in which the further substituent is a halogen, glycidylneodecanoate, hydroxymethyl, dimethylaminomethyl, 2-hydroxyethylmethylaminomethyl, t-butyl, sulphonate, styrene or benzoate.

9. A dye-sheet according to claim 8, in which the halogen is bromine.

10. A dye-sheet according to any of claims 5 to 9, wherein the hydrocarbyl group is (hydroxy)methyl, (hydroxy)ethyl or (hydroxy)butyl.

11. A dye-sheet according to claim 1, wherein the polymer is a copolymer formed of monomeric units according to formula 1 where Y is unsubstituted phenyl and monomeric units derived from maleic anhydride.

12. A dye sheet according to claim 1, in which the polymer comprises a copolymer formed from monomeric units according to formula 1 where Y is unsubstituted phenyl and monomeric units according to formula 1 where Y is an ester group of formula  $-\text{CO}_2\text{Z}$  wherein Z is an optionally substituted  $\text{C}_1$  to  $\text{C}_6$  hydrocarbyl group.

13. A dye-sheet according to claim 12, wherein the hydrocarbyl group is (hydroxy)ethyl, (hydroxy)propyl or (hydroxy)butyl.

14. A dye-sheet according to claim 1, wherein the polymer is selected from poly(parahydroxystyrene), poly(bromo-  
hydrocarbyl group is (hydroxy)ethyl, (hydroxy)propyl or (hydroxy)butyl.

15. A dye-sheet according to claim 1 wherein the substrate has a backcoat on the opposite side to the dye-coat.

10

16. A dye-sheet according to claim 1 for use in a light-induced thermal transfer process wherein a light absorbing material is present in the dye coat and/or a separate layer interposed between the dye coat and the substrate.

17. A thermal transfer printing dye-sheet which comprises a substrate having on one side, a dye coat comprising a binder and a thermally transferable dye wherein the binder comprises a polymer selected from the group consisting of:

a parahydroxystyrene homopolymer

a bromo-parahydroxystyrene homopolymer,

a copolymer of parahydroxystyrene and parahydroxystyrene further substituted with hydroxymethyl, diethylaminomethyl, 2-hydroxyethylmethylaminomethyl or t-butyl, or

a copolymer of parahydroxystyrene with or without a further substituent and any one of styrene, methyl (meth)acrylate, butyl (meth)acrylate and acrylic acid.

\* \* \* \* \*